

H. M. AND H. D. ABERNETHY.  
METHOD OF INSULATING ALUMINUM COVERED COPPER CONDUCTORS.  
APPLICATION FILED APR. 17, 1916.

1,323,236.

Patented Dec. 2, 1919.



Inventor

Harry M. Abernethy,  
& Harry D. Abernethy.

By Jas. L. Skidmore  
their attorney.

# UNITED STATES PATENT OFFICE.

HARRY M. ABERNETHY AND HARRY D. ABERNETHY, OF CLEVELAND, OHIO, ASSIGNEES  
OF ONE-HALF TO HARRY FULLER, OF EAST CLEVELAND, OHIO.

## METHOD OF INSULATING ALUMINUM-COVERED COPPER CONDUCTORS.

1,323,236.

Specification of Letters Patent.

Patented Dec. 2, 1919.

Application filed April 17, 1916. Serial No. 91,762.

To all whom it may concern:

Be it known that we, HARRY M. ABERNETHY and HARRY D. ABERNETHY, citizens of the United States, residing at Cleveland, 5 in the county of Cuyahoga and State of Ohio, have invented certain new and useful Improvements in Methods of Insulating Aluminum-Covered Copper Conductors, of which the following is a specification.

10 Our invention relates to an aluminum insulator and is especially designed for producing an insulator for copper, copper wire, or copper strips.

The main object of our invention is to 15 provide a simple, economical and efficient method of producing an aluminum insulator for copper, copper wire, or strips, which insulator possesses very high heat-resisting properties, and is practically fire-proof and 20 indestructible by the application of heat.

Another object of the invention is to provide an improved electrolyte solution in connection with a porous cup filled with 25 mercury for treating a copper wire or flat piece coated with aluminum, and by the use of a small voltage, and a small amount of electric current, produce an electrolytically deposited insulation that will withstand a puncture test of more than 1,000 volts.

30 A further object of this invention is to cover a copper wire conductor with a thin coating of aluminum, preferably by casting the aluminum around a copper billet, then rolling it into rods and drawing down to 35 wire sizes, then subjecting the wire to our improved electrolytic bath, thereby forming on the aluminum an insulation coating of such high resisting qualities that the wire may be melted from under the insulator, 40 thus leaving a tube.

The foregoing and such other objects as may appear from the ensuing description are attained by the novel features and arrangement of parts hereinafter more fully 45 described, illustrated in the accompanying drawing and particularly pointed out in the claims appended hereto, it being understood that slight changes in the form, proportions, and minor details of the structure shown 50 may be resorted to without departing from the spirit or sacrificing any of the advantages of the invention.

In the accompanying drawings it will be seen that the figure represents a diagram-

matic view of the improved device for carrying out our invention.

Numerals of reference are employed to designate the parts shown in the drawing.

In the embodiment of this invention as illustrated, the numeral 1 designates a receptacle of any suitable material which is filled with a solution composed of permanganate of potassium or sodium, water, and sulfuric acid, and within said receptacle is placed a porous cup 2, of any desirable material 6 filled with mercury, and while a coil of copper wire with a thin coating of aluminum, a straight piece, or flat piece may be suspended in the bath, constituting the anode of the system, we have shown a piece 65 of wire 3, of a serpentine form, suspended within the solution to which wire 3, is attached one terminal 4, of an electric generator 8, and attached to a piece of metal 5, located within the porous cup 2, which 70 contains the cathode of the system, is the second terminal 6, leading to the generator, and by the use of small voltage and current 75 a coating of insulation is formed on the aluminum coated wire 3, that will withstand 80 a puncture test of very high voltage, and thereby the thin coating of aluminum over the copper wire, or piece, is transformed 85 into an insulator of high heat-resisting substance which is substantially fireproof and almost indestructible by the application of 90 heat, and the wire may be melted from under or within the insulator and it still remains an efficient insulator.

It will be understood that long pieces of 90 the copper wire covered with a thin coating of aluminum may be drawn through a bath of the electrolytic solution hereinbefore referred to, whereby the said wire will be provided with an insulation possessing the 95 qualities herein stated.

It will be readily perceived that an electrical wire conductor thus produced possesses the advantage of taking up less space than the cotton or silk-covered wire commonly used in constructing magnets, motors and generators, besides a greater current carrying capacity, since so much of the aluminum as is not used for insulation purposes adds to the capacity of the copper 105 wire. Further advantages are apparent, not only from an economical standpoint, but from the ease in which a low voltage is

handled as compared with that of high tension, and we are enabled to obtain the full carrying capacity of the copper, and in a much less space as compared with the cotton 5 covered wire in general practice. Again, the high heat-resisting insulation quality is greatly appreciated by motor, generator and magnet builders, for the reason that any excess currents heats the wire thus charring 10 the insulation, which at once becomes a conductor causing short circuits and other interruptions.

Having thus described our invention what we claim, and desire to secure by Letters Patent is:—

1. The method of insulating a copper conductor covered with a thin coating of aluminum by subjecting said conductor to an electrolytic bath, composed of permanganate of 20 potassium, water and sulfuric acid, in connection with an electrical current, the said conductor forming the anode, and the cathode contained within a porous cup, thereby transforming said coating of aluminum into 25 an insulating substance.

2. The method of insulating an electrical conductor covered with a thin coating of aluminum, by subjecting the said conductor

to an electrolytic bath composed of permanganate of potassium, sulfuric acid and 30 water, in connection with an electric current of low voltage and a small amount of electric current, the said electric current passing from a generator to the anode and from a piece of metal carried by a porous 35 cup filled with mercury to a generator, thereby forming an insulation coating of high heat resisting substance entirely covering the aluminum coating.

3. The method of insulating an electrical 40 conductor covered with a thin coating of aluminum, by subjecting said conductor to an electrolytic solution within a container, in connection with an electric current of low voltage and a small amount of electric 45 current, passing the electric current from a generator to the anode and from a metal piece within a porous cup filled with mercury forming the cathode to the generator, whereby the outer part of said coating of aluminum is transformed into an insulation coating of high resistance entirely covering the surface of the aluminum. 50

HARRY M. ABERNETHY.  
HARRY D. ABERNETHY.